

Sept. 1, 1942.

M. GALLAGHER

2,294,744

WOODEN AGING BARREL

Filed Aug. 17, 1939

*Fig. 1*



*Fig. 2*



MILTON GALLAGHER  
INVENTOR

by Arthur J. Robert  
ATTORNEY

## UNITED STATES PATENT OFFICE

2,294,744

## WOODEN AGING BARREL

Milton Gallagher, Louisville, Ky., assignor to  
 Joseph E. Seagram & Sons, Inc., Shively, Ky.,  
 a corporation of Indiana

Application August 17, 1939, Serial No. 290,586

3 Claims. (Cl. 217—72)

This invention relates to wooden aging barrels, that is to say, barrels intended for the aging of liquids such as whiskey.

In aging whiskey, for example, considerable 5 outage, i. e., loss of whiskey, occurs due principally to evaporation from the barrel. While the rates at which evaporation proceeds from different sections of a wooden aging barrel are not known, one would normally expect them to be inversely proportional to the thickness of the 10 different sections, particularly since the overall outage of thick barrels is proportionately less than that of thin barrels during the same period of time. I have discovered, however, that this is not strictly true and that a substantial reduction in evaporation can be attained simply by sealing the barrel chimes, i. e., the bevelled ends of the staves, despite the fact that they present, as a whole, relatively remote evaporating surfaces and represent a very small part of the 20 total evaporating surface.

The principal object of my invention, therefore, is to provide a wooden aging barrel having its chimes coated with an impervious film.

The invention is illustrated in the accompanying drawing wherein:

Figure 1 is a perspective view of a fragmentary portion of one end of a barrel; and

Figure 2 is a section taken along line 2—2 of Figure 1.

A conventional whiskey barrel consists of a number of wooden staves 1 annularly arranged to form an open-ended cylinder having a central outward bilge. The cylinder has at each end a bevelled annular surface or "chime" 2, and, on its inner face adjacent each end, an annular recessed surface or "howel" 3, containing a centrally arranged annular groove or "croze" 4. Each end of the cylinder is closed by a head 5 having a marginal taper 6 terminating in a peripheral "bead" 7 which fits within the croze 4.

The staves 1 are cut so that the grain of the wood runs lengthwise of the staves whereby the ends thereof present end grain surfaces. During 45 the barrel-manufacturing process, after the cylinder is initially fabricated from the staves, it is fired on the inside to char the stave surfaces, machined to form the chimes, howels and crozes, and thereafter provided with the heads.

In accordance with my invention, the end grains of the staves, including the chimes 2, are sealed with a film 8 (see Figure 2) having a low 50 permeability preferably to both the gas and liquid phases of the barrel contents. I have found

in actual practice that, while a seal of this character covers a relatively small area, approximately 3 to 5% of the total outer surface area of the barrel, and, although it is rather distantly removed from the contents of the barrel, it, nevertheless, effects a substantial reduction in evaporation. For example, two sets of approximately 750 uncoated and 250 coated barrels having  $\frac{3}{4}$ " staves were weighed to determine the average weight loss per barrel over intervals of 5 and 10 months respectively, and such procedure repeated on barrels having  $1\frac{1}{8}$ " staves. The results thereof are tabulated as follows:

| Storage time | Stave thickness  | Average loss in weight per barrel |                  | Reduction in weight loss of coated barrels |
|--------------|------------------|-----------------------------------|------------------|--------------------------------------------|
|              |                  | Uncoated end grain                | Coated end grain |                                            |
| 5 months     | $\frac{3}{4}$ "  | 3.8                               | 3.3              | 13                                         |
| 10 months    | $\frac{3}{4}$ "  | 12.2                              | 10.9             | 11                                         |
| 5 months     | $1\frac{1}{8}$ " | 2.2                               | 1.8              | 18                                         |
| 10 months    | $1\frac{1}{8}$ " | 6.3                               | 5.2              | 17                                         |

Upon reference to this tabulation, it will be seen that the reduction in evaporation in the thinner barrels approximates 12 to 13% and in the thicker barrels 17 to 18%.

While various coating materials may be employed, good results can be obtained by using either a varnish composed of a synthetic resin dispersed in an organic solvent or a water-soluble compound having either sodium silicate or casein as the film-forming ingredient. If desired, a preformed Cellophane-like material comprising plasticizers and pigments, freed from solvents and volatile vehicles, may be attached to the end grain by the application of heat or by means of some adhesive such as shellac dispersed in pure grain alcohol.

The film may be applied before or after the barrel is completely fabricated. In some cases, the heat remaining in the barrel from the charring operation may be advantageously used to evaporate any volatile solvent in the film-forming material and thus effect a rapid drying of the film. Where the pores of the wood are large, it may be desirable to use a primer coat containing a suitable pigment such as aluminum powder for filling the pores and thus preparing the surface for the application of one or more following coats.

Having described my invention, I claim:

1. A wooden aging barrel having chimes and a coating of sealing material on said chimes, the

surfaces of the barrel being otherwise substantially free of sealing material.

2. A wooden aging barrel composed of staves in which the grain of the wood runs lengthwise and coating means for sealing the end grain of the staves, the surfaces of the staves being otherwise substantially free of sealing material.

3. An improvement in wooden-liquor-aging barrels composed of staves and heads, the staves

forming a cylinder having an inner wall croze adjacent to but spaced somewhat from each end, and the heads being jointed into the crozes, comprising: a coating of sealing material on the ends of the staves to reduce outage, the surfaces of the staves being otherwise substantially free of sealing material.

MILTON GALLAGHER.